

May 1, 1928.

1,668,349

E. G. BAUM

PAPER ARTICLE AND METHOD OF MANUFACTURE

Filed March 22, 1926



Inventor:  
Ewald G. Baum,  
by  
Wright Brown Daniels, Inc.  
Attys.

## UNITED STATES PATENT OFFICE.

EWALD G. BAUM, OF NATICK, MASSACHUSETTS, ASSIGNOR, BY MESNE ASSIGNMENTS, TO AMERICAN SEAL-KAP CORPORATION, OF NATICK, MASSACHUSETTS, A CORPORATION OF MASSACHUSETTS.

## PAPER ARTICLE AND METHOD OF MANUFACTURE.

Application filed March 22, 1926. Serial No. 96,503.

This invention relates to articles of cel-  
lulosic material and a method of manufac-  
ture, more especially of such articles formed  
up from paper sheets, as, for example, cer-  
5 tain forms of bottle caps or closures. More  
particularly it relates to such articles and  
their formation where resistance to deforma-  
tion in the presence of moisture is desirable  
or necessary.

10 It has been found that when such articles  
are formed by pressing sheets of paper out  
of their normally flat condition there is a  
strong tendency for such articles to flatten  
out somewhat under the action of moisture,  
15 even though the sheet material be quite  
thoroughly treated with waterproofing ma-  
terial, and where milk bottle caps are so  
made, these caps being provided with pour-  
ing lip housing portions, as shown, for ex-  
20 ample, in my Reissue Patent No. 15,491  
dated November 21, 1922, for bottle caps,  
this tendency, if not counteracted, causes  
the marginal portions thereof to flare so  
that they do not properly engage the bot-  
25 tle. The caps then do not hold to the bot-  
tles with sufficient tenacity and the contents  
are not always completely sealed.

By the method of the present invention,  
however, the structure of the paper is so  
30 modified over at least those portions where  
flattening would be likely to be detrimental,  
that such flattening tendency is quite ef-  
fectually prevented. In general the method  
comprises a preliminary treatment of the  
35 paper by which the cellulosic fibers are  
swelled and softened and by which the de-  
sired waterproofing compounds are incor-  
porated therein prior to the forming of the  
paper into the article, and after this pre-  
40 liminary treatment the subjection of the ma-  
terial, preferably in the process of forma-  
tion, to such heavy pressure, at least over  
that portion or portions where flattening is  
to be prevented, that the fibers are compacted  
45 together and the fibers of successive over-  
lapping layers interfelted so as to form with  
the waterproofing agent a dense, horn like,  
translucent structure in the desired shape  
quite different from the structure of the  
50 paper sheet before being subjected to this  
pressure.

For a more complete understanding of this  
invention reference may be had to the ac-  
companying drawings showing the applica-  
tion of the method to a form of a milk bot-  
tle cap somewhat like that shown in my re-  
55 issued patent hereinbefore referred to. In  
these drawings,

Figure 1 is a plan of a blank from which  
the cap is to be formed.

Figures 2, 3, 4 and 5 are detail sections  
showing successive positions of the dies  
relative to each other and to the blank as it  
is being formed into a cap.

Figures 6 and 7 are elevation and plan  
views, respectively, of a partially formed  
cap corresponding to that illustrated in Fig-  
ure 4.

Figure 8 is a detail section on line 8—8 of  
Figure 6.

Figure 9 is a side elevation of a fully  
formed cap.

Figure 10 is a detail section on line 10—10  
of Figure 9.

The paper stock employed for this process  
should have high absorptive qualities and  
should be of uniform thickness and of a  
strength as near as possible the same across  
the sheet as in its lengthwise direction. The  
paper is blanked out to the form required  
80 to make up the article and either before or  
after the blanking operation, is subjected  
to the following steps.

First, it is treated with water which it  
should be capable of absorbing freely, the  
water being applied to the paper under such  
conditions of time pressure and temperature  
as are found most suitable with the particu-  
lar stock being employed. The warmer the  
water the easier the paper absorbs it under  
ordinary conditions. If the water is warm  
the pressure or time of treatment or both  
may be reduced, or the treatment may be  
prolonged under lower pressure or tempera-  
ture conditions or both. The treatment  
90 should be sufficiently thorough, however, to  
cause the cellulosic fibers of the paper to  
swell and soften to a material extent. The  
moistened paper should be allowed to stand  
a sufficient time so that the moisture be-  
comes uniformly spread through its tex-  
ture. Ordinarily but a few minutes is neces-  
100

sary for this, the time necessary depending largely on the particular paper stock being employed and somewhat also on the moistening methods which may have been used.

- 5 The paper should then be passed through a waterproofing compound preferably at an elevated temperature. The compound which has been found most suitable in practice comprises waxes, such, for example, as
- 10 paraffin preferably with the addition of a small amount of hardening wax such as carnauba or Montan wax. The particular composition of the wax may be varied to suit the product and also somewhat to suit
- 15 the stock being treated. When the moistened and swollen paper passes into this bath of wax which should be at a temperature above 212° F., as for example from approximately 235° F. to 240° F., a portion
- 20 of the water in the material is converted into steam and escapes and as the paper passes out from the melted wax the condensation of steam which may remain in the paper draws in the melted wax so as to impregnate its fibrous structure without destroying its tensile strength, and to fill the intercellular spaces of the paper without however causing the fibers to be shrunk and contracted to their substantially dry condition.
- 25
- 30

After the sheet material is treated with the wax it is preferable to permit it to stand for some hours, say 24 or more, in a closed container, the material then cooling and seasoning or tempering. When removed from these containers it is in condition for the forming operation. In the case of the formation of the bottle cap of the type hereinbefore described the operations to be car-

- 35 ried out are shown somewhat diagrammatically in the drawings. A waxed and tempered blank 1 is placed upon the die member 10, shown in Figures 2 to 5, and the die member 11 is brought down on its central portion as at 2, the blank being thus held in position for the further forming operations. Next the die member 12 is brought down against the upper face of the blank, pressing it against the outer portion 13 of
- 40 the die member 10. Next the die member 14 is moved upwardly, as shown in Figure 4, forming up the upstanding wall 15 which is to engage the inner wall of the milk bottle above the usual annular ledge therein on
- 45 which the usual disk of cardboard is placed. Next the outer die member 16 is brought downwardly to form the outer margin of the blank into the downwardly extending portion 17, shown best in Figure 9, which
- 50 bears against the outer face of the bottle pouring lip. The pressure exerted on the material by these dies is very considerable, being on the order of from 6,000 to 10,000 pounds per square inch for waxed paper
- 55 approximately .028 inch thick or .022 inch

thick before being softened and waxed, and the clearances between the die members 12, 14 and 16 are so proportioned that substantially this pressure is exerted on the material therebetween when the cap is being formed.

It will be noted that since the maximum diameter of the finished cap is very much smaller than that of the blank from which it is formed, the material in the inner upstanding and in the outer downwardly extending portions 15 and 17, respectively, must be gathered together in overlapping layers, and where the material is treated as hereinbefore described prior to the forming operations this heavy pressure causes these overlapping portions to be pressed together resulting in more or less interfelting of the fibers in the contacting layers and compacting the fibers and the wax into a dense, horn-like structure which is highly resistant to the action of moisture.

Where articles of paper are formed up by pressing from flat sheet material there is a strong tendency for overlapping layers to separate somewhat so that the material tends to flatten after formation, this tendency being particularly noticeable when the articles are subjected to moisture conditions. If this should be permitted in the case of a bottle cap of the type shown, it would result in the outer pouring lip housing wall flaring so that its lower edge would not properly engage the outer side of the bottle and would also result in the inner wall engaging the inner wall of the bottle drawing away from close contact with the bottle so that the sealing qualities of the cap would be very greatly impaired and its removal from the bottle would be rendered too easy for security. By the treatment herein outlined, however, this pouring lip housing, which is of general channel shape in section, is maintained in proper condition with the opposite walls thereof in the form in which they are produced by the dieing operation. It has been found in practice that such a cap may be subjected to water for an indefinite time without showing any tendency for flattening of the cap or flaring of these walls to occur.

Preferably, though not necessarily, the upper portion of the pouring lip housing has radial corrugations since this construction produces added resiliency to the pouring lip housing portion so that it may be pressed over the pouring lip and tightly engage it on opposite sides. Preferably also the heavy pressure is applied to substantially the entire area of the cap including its central bore-covering portion, the upstanding wall portions 20 which are formed to engage the inner wall of the bottle beneath the usual disk-receiving annular ledge, and the annular portion 21 which is formed to seat on the upper face of this

annular ledge. This heavy pressure produces a stiffening of the material, which is of advantage, and it also renders it more nearly waterproof.

5 In Figures 6, 7 and 8 is illustrated the manner in which the material is gathered together in overlapping folds in the portion 17 of the cap, this being shown in the condition wherein this portion of the cap has not been 10 completely formed, while Figure 10 illustrates in section the condition of this portion of the cap after it has been subjected to the heavy pressure so that it has been reduced to a substantially homogeneous, translucent, 15 horn-like structure of substantially uniform thickness with the fibrous material of the overlapping layers felted together. This horn-like structure of the material can not be produced by the use of a water treatment 20 alone, apparently the wax or its equivalent waterproofing material being necessary to produce the interfelting of the fibers under the pressure to which they are subjected according to this method. This material also 25 serves an important function in the formation of the wall portions 15 and 17 of the cap in that it acts as a lubricant between the die members and the sheet material and prevents these members from tearing the material due 30 to their severe rubbing effect thereon during the forming operation. It also acts as a binder for the fibers and the layers in the finished product.

Having thus described this invention it 35 will be evident that various modifications and changes might be made therein without departing from its spirit or scope as defined by the appended claims.

I claim:

40 1. An article formed up from sheet cellulosic material containing a waterproofing agent and having portions of the sheet in folded overlapping relation, said portions being compressed to substantially uniform 45 thickness and presenting a dense horn-like structure resistant to opening up when subjected to moisture.

2. An article comprising sheet cellulosic material having portions thereof in overlapping relation, said portions presenting a dense, horny, interfelting structure resistant to separation of the overlapping portions when subjected to moisture.

50 3. An article formed up from waxed sheet cellulosic material and having a portion comprising folded layers of such sheet material interfelting and compressed to a translucent, 55 horn-like condition.

4. An article formed up from waxed sheet 60 cellulosic material and having a portion comprising folded layers of such sheet, such portion being formed into a dense, horny structure retaining its folded condition indefinitely when subjected to moisture.

5. An article formed up from a sheet of 65 waxed paper and having a portion comprising folded layers of such sheet, said portion being compressed to form a dense, horny structure retaining its folded condition indefinitely when subjected to moisture. 70

6. A milk bottle cap having a bore-covering portion terminating in an upstanding portion engageable with the inner wall of a milk bottle below the usual disk-receiving annular ledge therein, a portion formed to 75 overlie said ledge, a portion upstanding from said ledge-engaging portion to engage the inner wall of the bottle above said ledge, and a marginal downwardly turned portion engageable with the outer wall of the bottle, 80 said upstanding and downwardly turned portions presenting dense structure resistant to deformation when subjected to moisture.

7. A milk bottle cap of waxed paper having a bore-covering portion terminating in 85 an upstanding portion engageable with the inner wall of a milk bottle below the usual disk-receiving annular ledge therein, a portion formed to overlie said ledge, a portion upstanding from said ledge-engaging portion to engage the inner wall of the bottle above said ledge, and a marginal downwardly turned portion engageable with the outer wall of the bottle, said upstanding and 90 downturned portions comprising layers of 95 the waxed paper folded together and compacted to a dense, translucent, horn-like condition resistant to unfolding in the presence of moisture.

8. A bottle cap having a pouring lip housing engageable with opposite sides of the bottle wall, the wall-engaging portions comprising folded layers of interfelting sheet material compressed to a translucent horn-like condition resistant to deformation in the 100 presence of moisture.

9. The step which comprises forming a waxed blank of softened sheet cellulosic material into an article under sufficient pressure to convert such material over at least a portion of the article into a dense, compact, 110 horn-like material.

10. The step in the process of forming a waxed blank of moistened cellulosic sheet material into an article having portions of 115 the sheet in folded overlapping relation which comprises subjecting said portions to pressure sufficiently heavy to compact them to substantially homogeneous rigid horn-like structure of substantially uniform thickness. 120

11. The method which comprises swelling and softening a blank of fibrous sheet material, incorporating wax therein, and then forming an article from the blank thus treated under pressure sufficiently heavy to compact the material together into a dense, 125 horny condition.

12. The method which comprises treating

a fibrous blank with water, passing the wet blank through a liquid wax heated to a temperature above 212° F. and thereby vaporizing a portion of the water from said blank  
6 and saturating the blank with the wax, permitting the blank thus treated to temper, and then forming said blank to the desired

shape under pressure sufficiently heavy to compact and densify at least a portion of the blank to a dense, rigid, horn-like condition. <sup>10</sup>  
In testimony whereof I have affixed my signature.

EWALD G. BAUM.